

June 21, 1932.

E. W. DAVIS

1,863,622

PROCESS OF PRODUCING IRON OR STEEL DIRECTLY FROM THE ORE AND  
CONTROLLING THE SULPHUR CONTENT THEREOF

Filed July 28, 1928

5 Sheets-Sheet 1

*Fig. 1.*



Inventor

*Edward W. Davis*

By his Attorneys

*Hogsett & Meany*

June 21, 1932.

E. W. DAVIS

1,863,622

PROCESS OF PRODUCING IRON OR STEEL DIRECTLY FROM THE ORE AND  
CONTROLLING THE SULPHUR CONTENT THEREOF

Filed July 28, 1928

5 Sheets-Sheet 2

Fig. 2.



Inventor  
Edward W. Davis

By his Attorney,  
Hogsett & Meany

June 21, 1932.

E. W. DAVIS

1,863,622

PROCESS OF PRODUCING IRON OR STEEL DIRECTLY FROM THE ORE AND  
CONTROLLING THE SULPHUR CONTENT THEREOF

Filed July 28, 1928

5 Sheets-Sheet 3

Fig. 3.



Inventor  
Edward W. Davis.

By his Attorney's  
Hogness & Neary

June 21, 1932.

E. W. DAVIS

1,863,622

PROCESS OF PRODUCING IRON OR STEEL DIRECTLY FROM THE ORE AND

CONTROLLING THE SULPHUR CONTENT THEREOF

Filed July 28, 1928

5 Sheets-Sheet 4

Fig. A



Inventor

Edward W. Davis

By his Attorneys

Hoguet & Neary.

June 21, 1932.

E. W. DAVIS

1,863,622

PROCESS OF PRODUCING IRON OR STEEL DIRECTLY FROM THE ORE AND  
CONTROLLING THE SULPHUR CONTENT THEREOF

Filed July 28, 1928

5 Sheets-Sheet 5

Fig. 5.



Inventor

Edward W. Davis

By his Attorneys.

Hogers & Neary

## UNITED STATES PATENT OFFICE

EDWARD W. DAVIS, OF MINNEAPOLIS, MINNESOTA, ASSIGNOR TO DAVIS STEEL PROCESS CORPORATION, A CORPORATION OF DELAWARE

PROCESS OF PRODUCING IRON OR STEEL DIRECTLY FROM THE ORE AND CONTROLLING THE SULPHUR CONTENT THEREOF

Application filed July 28, 1928. Serial No. 296,019.

This invention relates to a process of reducing iron from its ores in which the reduction of the ore and the production therefrom of iron or steel take place in a furnace of the 5 reverberatory type, and in particular to a process for controlling the sulphur content of the metal product.

In my co-pending application Serial No. 293,491, filed July 17, 1928, I have described a 10 process for the production of pig iron or steel by the direct reduction of ores in furnaces of the reverberatory type wherein an economic recovery of the iron content of the ore or other iron-bearing material treated is made 15 possible by properly utilizing the ability of carbon to unite very rapidly with reduced iron when suitable temperatures are employed. The present invention contemplates, according to a preferred embodiment, the use 20 of the rule disclosed in the above-mentioned application in conjunction with certain new rules or principles of operation whereby not only is it made possible to effect an optimum recovery of the metal content of the ore that is 25 being smelted, but also to control the sulphur content of the metal product.

This process rises from the discovery of certain relationships existing between the percentage of sulphur retained by the metal 30 and certain operating factors of the smelting operation, and represents a considerable modification of and departure from the principles hitherto considered as governing the production of low sulphur metal in smelting 35 operations. According to the smelting process heretofore generally employed for producing fluid metal directly from the ore, that is, by means of the blast furnace, and as well, according to the proposals heretofore made for reducing ores and producing 40 fluid metal therefrom in furnaces of the reverberatory type, it has been considered essential, in the production of low sulphur metal, so to proportion the fluxing constituents of the charge as to produce a strongly 45 basic slag. I have discovered, however, that low sulphur metal may be produced in reverberatory smelting processes using acid and neutral slags with the same facility 50 as basic slags, provided the iron oxide con-

tent of the slag is kept below a certain limiting percentage. I have also ascertained that this limiting percentage of iron oxide in the slag is variable with respect to the nature of the slag and the percentage of sulphur desired in the finished product. My invention makes it unnecessary therefore to limit the slag to a particular type as heretofore was believed to be the case. 55

My investigations show that with a given 60 furnace, working on a given ore and with a given method of feeding, the sulphur content of the metal produced can be decreased by (1) increasing the temperature of the furnace; (2) increasing the carbon content of the 65 charge; and (3) increasing the basicity of the slag-forming ingredients of the charge.

In order to illustrate the principles of my invention I am indicating graphically in the 70 appended drawings the relationships which I have found to exist between the sulphur content of the metal and the iron oxide content of the slag, and between the basicity or acidity of the slag, the iron oxide of the slag and the sulphur content of the metal, as well 75 as the relationship between the sulphur of the metal and the carbon-iron ratio of the charge.

In the drawings, Fig. 1 is a graph representing the results of many tests showing 80 the relation between the sulphur content of the metal and the iron content of the slag;

Fig. 2 shows a series of curves indicating the 85 relation that it is necessary to maintain between acidity and iron content of the slag in order to produce metal analyzing .03%, .05% and .08% sulphur;

Fig. 3 represents a series of curves showing 90 the effect of change of the coal-iron ratio of the charge when operating under acid conditions with a 65% acid slag.

Fig. 4 represents a series of curves showing 95 the effect of change of the coal-iron ratio of the charge when operating under basic conditions and with a slag containing approximately four parts lime (CaO) to 3½ parts silica (SiO<sub>2</sub>).

Fig. 5 represents a series of curves showing 100 the effect of change of the coal-iron ratio of the charge when operating under acid con-

ditions with a 65% acid slag and with a different method of feeding the charge than was employed in obtaining the results indicated in Figs. 3 and 4.

5 The points indicated on Fig. 1 represent results, as regards iron content of the slag and sulphur content of the metal, obtained in smelting operations carried out with a magnetite ore containing about 60% iron, about 10 13.5% silica and small amounts of lime, magnesia and alumina, and with the amounts and character of fluxing additions varied all the way from strongly acid conditions on the one hand to strongly basic conditions on the 15 other. The graphical representation of these results clearly shows that an acid slag must be lower in iron for a given sulphur analysis than a basic slag. The more basic the slag is, the more iron it can contain for a given 20 sulphur content of the metal. This is indicated on the graph by the two limit curves, the lower one being for strongly basic slags, i. e., 65% base, and the upper one for strongly acid slags, i. e., 70% acid. From these results 25 it is apparent that as the iron is reduced in the slag the sulphur is eliminated from the metal. A change of 1% in the iron content of the slag makes a considerable difference in the sulphur content of the metal, but this difference is much greater with the acid slags than with the basic slags.

The data from which the curves shown in Figs. 2, 3, 4 and 5 were plotted was obtained 30 from the results of smelting operations carried on with the magnetite ore above mentioned. All of the smelting operations, the results of which were used in making up the curves shown in Figs. 1, 2, 3 and 4, were conducted as "batch" operations at temperatures 35 of around 1500° C., during the earlier portion of the reducing stage and before any substantial melting takes place, and at approximately 1600° C. during the later stage when the reduction is completed and carburizing and 40 melting of the reduced metal takes place. By a "batch" operation, I mean a smelting operation in which the ore, carbonaceous reducing agent, and all or a part of the fluxing additions sufficient to form a complete charge are 45 introduced at one time and such charge is melted down and tapped without making continuous or periodic additions of ore or carbon during the operation.

50 All of these temperatures were recorded by 55 use of an optical pyrometer sighted on the surface of the molten bath and are intended merely to serve as an indication but not as a measurement of the actual temperature of the carburization reaction itself or other reactions taking place in the smelting zone. With different ores and with different carbon content of the charge, and/or different amount and character of slag-forming materials present, the temperature at which the 60 65 furnace should be maintained will depend

upon the changed conditions within the furnace and will vary with such changes.

In the smelting operations, the results of which were used in making up the curves shown in Fig. 5, the charge was fed substantially continuously through openings in the roof of an acid-lined reverberatory furnace. Sufficient of the mixture was introduced to build up and maintain a body of charge with a relatively large sloping surface exposed to the heating action of the flame passing through the furnace; thus permitting the reduced metal as it carburized and melted to run into the bath which formed at the bottom.

70 75 80 The carbonaceous material used in all of these smelting operations was Pocahontas coal crushed to -6 mesh size.

In the light of the foregoing, it will be seen that my investigations have made it possible 85 to greatly increase the flexibility of the smelting process. By proper correlation of the various factors of temperature, basicity or acidity of the slag and carbon-iron ratio of the charge, I have made it possible to control the sulphur content of the metal product within a wide range and to obtain low sulphur metal 90 by carrying out the ore reduction under basic, acid or neutral conditions, as desired.

95 For example, let us assume that it is desired to obtain a metal product with a sulphur content of .03% and that the smelting operation is to be carried out in an acid-lined furnace, as a "batch" operation. The charge will then be made up with proportions of 100 coal, ore and fluxing additions so chosen that when the ore has become reduced and the reduced metal has carburized and melted down into a fluid state, a product of the desired sulphur content will be produced. To be specific, if it is proposed to use a slag consisting of 60% acid materials such as silica, and 40% basic materials such as lime, reference to Fig. 2, will show that in order to produce metal having .03% sulphur the iron content of the slag should be about 1.15% with a 60% acid slag. The coal-iron ratio of the charge will then be so chosen as to produce a slag having an iron content of about 1.15%. In the example given, a ratio of 66 110 parts coal to 100 parts iron in the charge 115 would be required.

In carrying out my invention I propose to use the existing types of reverberatory furnaces, such for example, as the ordinary open hearth furnace used in steel making operations. Any of the ordinary forms of iron ore may be used as well as flue dust, gas washer sludge, pyrites, cinder, mill scale, turnings, borings and other mill and machine shop waste. The invention is particularly applicable to the treatment of the fine oxide ores and other iron oxide materials which it has heretofore been impossible to handle economically in a blast furnace without resorting to beneficiating operations.

It will be understood that the method of feeding is a factor to be considered and that different results as regards sulphur content of the metal and iron content of the slag 5 will be obtained in a "batch" operation than in a smelting operation in which the charge is fed continuously or substantially continuously. This is illustrated by comparing the results shown in Fig. 3 with the results in-

10 dicated in Fig. 5. These different results may be explained in part at least as due to differences in the ratio of surface of the charge exposed to the heating gases, and to differences in the time factor. The relation 15 which these respective constituents of the metal product and the slag bear to one another is, however, substantially the same irrespective of the method of feeding so that the rules as to correlation apply to all methods of feeding.

As a specific example of the batch method of smelting, the following is set forth: a charge was made up of 2926 lbs. of magnetite in finely divided form and analyzing about 25 60% iron, 13.5% silica and small amounts of lime, magnesia and alumina, etc.; 975 lbs. Pocahontas coal crushed to -6 mesh size and 900 lbs. of limestone crushed to -4 mesh size. The coal was mixed with 2576 lbs. of magnetite, sufficient water being added to prevent dust losses. The mixture was evenly distributed over the hearth of an open hearth furnace and covered with the remainder of the ore mixed with a like amount by weight 30 of limestone. The rest of the limestone was added at intervals during the smelting operation. The temperature was brought up to about 1500° C., and held there for about three hours. The reduction of the ore to a 35 considerable depth in the charge was substantially completed at the end of this period, whereupon the temperature was then raised to about 1600° C. and held there for about ten hours or until the reduced metal 40 had become carburized and melted, when the metal was tapped. The slag at the end of the operation analyzed 1.63% iron and the metal analyzed 3.01% carbon, 0.016% sulphur, 0.057% phosphorus and 0.41% silicon.

45 While a cover was used in carrying out the above operation, it is not essential if the heating is carried out under the proper control as to temperature so that advantage is taken of the ability of carbon to unite very rapidly with reduced iron as described in my co-pending application hereinbefore mentioned. That is to say, by operating at a temperature above that at which the rate of carburization changes very abruptly and 50 becomes relatively great.

55 I find that in carrying out the process as a batch operation it is desirable to so control the time and rate of heating during the early portions of the reducing stage that the evolution of gases which attends the reducing op-

eration will not become so rapid as to cause "spouting" or local eruptions in the charge. This spouting is disadvantageous not only because of the increased difficulty of control of the iron content of the slag, but also because of the fact that molten or partially fused material is carried over into the checkers with consequent stoppage of the passages.

70 When operating with continuous or substantially continuous feeding of the charge as hereinbefore mentioned, the temperature may be maintained at any point desired throughout the smelting operation since the conditions which tend to produce spouting, namely a relatively large body of unreduced material upon which is superimposed a body of molten metal and slag which tends to penetrate into the underlying charge and cause unduly rapid reduction of the charge 75 and evolution of gas to take place, are absent.

80 As illustrative of the effect of varying the ratio of carbon to iron in the charge on the sulphur content of the metal when carrying out the smelting operation with substantially 85 continuous feeding of the charge as above mentioned, the following examples are given:

85 Let us assume that an operating temperature of 1600° C. is being maintained and that a magnetite ore assaying 60% iron and 12% 90 silica, with small amounts of lime, magnesia, etc., is used. With a charge of the following proportions: 100 lbs. of ore, 33 lbs. of Pocahontas coal and 7 lbs. of limestone, the metal will contain ordinarily about .25% 95 sulphur. If the weight of the coal used in the charge is increased to 43 lbs. per 100 lbs. of ore, the sulphur in the metal will be reduced to about .15% sulphur. If a charge of 100 lbs. of ore, 43 lbs. of Pocahontas coal 100 and 25 lbs. of limestone is used, the metal will contain about .05% sulphur.

105 Instead of varying the carbon content of the charge while maintaining the other factors constant, it may be desirable to vary the 110 temperature, the nature and chemical composition of the slag, or the method of feeding, while maintaining the other factors constant, or to vary more than one or all of the factors. This will be determined by the economic and practical considerations which confront the particular operator, such as availability and cost of fluxing materials and fuels, chemical composition and structure of the ore, the type of furnace available and the 115 limit determined upon for the sulphur content of the product.

120 It may also be desired to vary the conditions during the course of the smelting operation and, if so, the rules hereinbefore set 125 forth make it possible to effect any desired regulation and control of the sulphur. For example, if the furnace is being operated at 1600° C. and with a neutral slag, a satisfactory method for decreasing the sulphur con- 130

tent of the metal is to increase the carbon content of the charge, since an increase in temperature or basicity of the charge will in this case only slightly decrease the sulphur content of the metal and may be injurious to the furnace. However, if the furnace is being operated at 1500° C., and with a neutral slag, the best method is usually to increase the temperature, as this not only decreases the sulphur content of the metal but also increases the melting capacity of the furnace. If the furnace is being operated with a strongly acid slag, a decrease in the sulphur content of the metal can be produced by increasing the basicity of the slag-forming ingredients of the charge. If a variety of fuel are available, the sulphur content of the metal can ordinarily be reduced by using a more graphitic form of carbon or fuels that are low in sulphur.

What I claim is:

1. In a process of producing fluid iron or steel directly from the ore by smelting a mixture of ore, carbon and fluxing materials with an oxidizing flame in a furnace of the reverberatory type, and in which the slag-forming constituents of the charge are so adjusted as to kind and amount as to form a slag containing insufficient basic constituents to combine with all of the sulphur that is to be removed, the step which comprises regulating the sulphur content of the metal produced by controlling the iron oxide content of the slag.
  2. In a process of producing fluid iron or steel directly from the ore by smelting a mixture of ore, carbon and fluxing materials with an oxidizing flame in a furnace of the reverberatory type, and in which the slag-forming constituents of the charge are so adjusted as to kind and amount as to form an acid slag containing insufficient basic constituents to combine with all of the sulphur that is to be removed, the step which comprises regulating the sulphur content of the metal produced by controlling the iron oxide content of the slag.
  3. In a process of producing fluid iron or steel directly from the ore by smelting a mixture of ore, carbon and fluxing materials with an oxidizing flame in a furnace of the reverberatory type, and in which the slag-forming constituents of the charge are so adjusted as to kind and amount as to form a basic slag containing insufficient basic constituents to combine with all of the sulphur that is to be removed, the step which comprises regulating the sulphur content of the metal produced by controlling the iron oxide content of the slag.
- 60 In testimony whereof, I have signed my name to this specification this 12th day of July, 1928.

EDWARD W. DAVIS.